

## UNITED STATES PATENT OFFICE

2,107,282

METHOD OF REMELTING AND REFINING  
MAGNESIUM AND LIGHT METAL ALLOYS  
CONTAINING MAGNESIUMAdolf Beck, Bitterfeld, Germany, assignor, by  
mesne assignments, to Magnesium Develop-  
ment Corporation, a corporation of DelawareNo Drawing. Application July 10, 1936, Serial  
No. 90,006. In Germany July 19, 1935

7 Claims. (Cl. 75—67)

This invention relates to a method of re-melting and refining magnesium and light metal alloys containing magnesium, more particularly high percentage magnesium-base alloys.

5 It has of late frequently been asserted that the saline melts employed for re-melting and refining magnesium and high percentage magnesium-base alloys, and containing, besides chlorides of the alkaline-earth metals, and on occasion of the  
10 alkali metals, additions of thickening or inspissating substances such as metal oxides or fluorides, melt only at temperatures at which the metal to be treated is already in a molten state, and that, in consequence, the tendency of the  
15 molten metal to relatively extensive oxidation cannot be entirely suppressed by the fluxing agent, which was supplied in the form of powder, in the bottom of the crucible, or strewn over the metal to be melted, since at the melting tempera-  
20 ture of the metal said fluxing agent was still unmolten and thus incapable of protecting the metal from oxidation by the formation of a coherent layer.

In order to obviate this drawback, it has been  
25 proposed to employ fluxes fusing below the melting point of the metal under treatment, the intention being for the flux, by melting first, to form a protective cover on the metal which has not yet melted, or is in course of melting. How-  
30 ever, in the case of these fluxes, which contain no inspissating agents, or only small amounts thereof, the thickening effect obtainable by the addition of such inspissating agents is of course absent, that is to say, owing to their high fluidity,  
35 or low surface tension at higher temperature—even at such as are only about 100—150° C. above the melting point of the metals under treatment—it is impossible to obtain a clean separation of the flux from the metallic regulus after  
40 the treatment is finished; and there is therefore always a risk of traces of flux being entrained by, or included in, the metal, on pouring, such traces afterwards giving rise to the corrosion phenomena which, for a long time, made the  
45 commercial employment of magnesium or its alloys impossible.

Nevertheless, by suitably modifying the known process of re-melting and refining light metals, with the aid of chloride fluxes containing inspissating or thickening agents, it is possible, on the one hand, to prevent any extensive oxidation of the metal during re-melting and, on the other, to secure a clean separation of the flux from the treated metal, under all conditions.

55 According to the present invention the known

process of melting and refining magnesium and light metal alloys containing magnesium is modified with a view to ensuring an efficient protection, from oxidation, of the metal to be treated, during the melting stage by the presence of an 5 easily fusible flux, whilst at the same retaining the advantages resulting from the use of inspissated fluxes, namely complete removal of the flux from the metal after completion of the refining operation.

To this end, according to the invention, the metal under treatment is first melted down in the presence of a thinly fluid, i. e., non-inspissated, flux containing one or more chlorides and having a melting point which is not substantially 10 higher than that of the metal, and which on occasion, may be substantially below the latter. Substances which have been found particularly suitable for this purpose are anhydrous carnallite, or mixtures still richer in potassium chloride such as for example,  $2\text{KCl} \cdot \text{MgCl}_2$ , having a melting point of 580° C. or less, that is to say, at least about 70° C. below the melting point of pure magnesium. The desired effect may, however, also be obtained with pure anhydrous magnesium chloride, containing additions of chlorides other than potassium chloride, tending to lower the melting point.

In carrying out the invention, it is immaterial whether, by using a somewhat larger quantity 20 of the flux, the metal melts down into a sump 30 of flux in the bottom of the crucible, or whether the flux be strewn as powder, over the metal to be melted, or added by degrees in accordance with the progress of the melting operation. In 35 any event, the readily fusible flux will afford extensive protection to the metal against substantial oxidation during the melting operation. As soon as a substantial sump of molten metal has formed, further portions of flux may be applied, 40 as a mobile protective coating, to the surface of the metal, in order to protect this portion of the metal from any extensive oxidation.

When the whole of the metal under treatment is in a molten state, the melt is energetically 45 stirred in the usual manner, in order to enable the flux to take up any impurities contained in the metal. This operation can be carried out, without substantial oxidation of the metal, at temperatures below about 800° C. During this 50 cleansing action, the known inspissating or thickening agents may be added to the metal bath, in suitable amounts for inspissating the flux already present, or alternatively, suitable amounts (according to circumstances) may be 55

added, of a flux of fundamentally the same composition as that of the known fluxes containing inspissating or thickening agents, but preferably with a larger proportion of these latter than usual, in order that, in being contacted with the mobile flux already present in the metal bath, the newly added flux may also have an inspissating effect thereon. The known mixtures of magnesium chloride with magnesium fluoride, calcium fluoride and/or magnesium oxide, or of calcium chloride with magnesium fluoride, are specially suitable for this purpose.

After the stirring has been completed, which, in the case of small units, usually does not take any longer than about 1 minute, but may be continued for a considerable time, or be frequently repeated, if necessary, in accordance with the amount of impurities contained in the metal, the melt is covered, in known manner, with a protective layer of a flux containing a normal proportion of inspissating agents, and is then heated to considerably above the pouring temperature for the purpose of separating the final traces of agglomerated flux from the metallic regulus. The metal is thereupon poured, on occasion after cooling to pouring temperature, and the coherent solid covering of flux is held back by suitable means such as rakes or the like.

The fluxes employed in carrying out the invention may consist merely of mixtures of the ingredients. Sometimes, however, it is preferable to pre-melt the ingredients down together and to crush the mass after solidification, because this method ensures more intimate mingling of the components. If desired, salts of a metal which is already present in the alloy, may be incorporated with the flux, in known manner, in order to prevent the said metal being washed out during the treatment with the flux. The fluxes may moreover contain additions which become reduced by the metallic melt and enter into the metal or alloy.

*Example*

A cast-iron crucible is first strewn with a thin fluxing layer consisting of anhydrous carnallite, and is then charged with about 30 kgs. of a high percentage magnesium alloy, in the form of ingots, and heated. Directly incipient melting is observable, further quantities of the same flux are strewn in small portions over the still solid lumps of metal, and, after a metal sump has formed, the surface of this also is covered with a little anhydrous carnallite. The total amount of flux used, up to the end of the melting process, is 200 grammes.

When the temperature reaches 720° C. the metal is thoroughly stirred for about a minute with a stirring rod, and, at the same time, a total amount of 250 grammes of a flux, consisting of:

|                             | Per cent |
|-----------------------------|----------|
| Anhydrous MgCl <sub>2</sub> | 70       |
| MgO                         | 10       |
| CaF <sub>2</sub>            | 20       |

is strewn, in small portions, over the surface. After completing the stirring, the surface of the metal is evenly covered, by strewing, with about 150 grammes of a flux composed of:

|                   | Per cent |
|-------------------|----------|
| MgCl <sub>2</sub> | 80       |
| MgO               | 10       |
| CaF <sub>2</sub>  | 10       |

which soon sinters in the form of a coherent,

viscous layer. Under this layer, the contents of the crucible are heated at about 850° C. for a short time, then cooled to the pouring temperature of 760° C. and poured in known manner.

I claim:

1. A method of re-melting and refining magnesium and light metal alloys containing magnesium and more particularly high percentage magnesium-base alloys, which comprises melting the metal in the presence of a thinly fluid saline flux having a melting point not substantially exceeding the melting temperature of the metal, then increasing the temperature of the metal, then stirring the metal at such elevated temperature with the said flux while adding a thickening agent in a quantity sufficient to cause inspissation of the flux already present, so as to cause said flux to combine with said inspissating agent and with the non-metallic impurities contained in the metal, and finally pouring said metal.

2. A method of re-melting and refining magnesium and light metal alloys containing magnesium and more particularly high percentage magnesium-base alloys, which comprises melting the metal in the presence of a thinly fluid saline flux having a melting point not substantially exceeding the melting temperature of the metal, then increasing the temperature of the metal, then stirring the metal at such elevated temperature with the said flux while progressively adding portions of a thickening agent in an aggregate quantity sufficient to cause inspissation of the flux already present, so as to cause said flux to combine with said inspissating agent and with the non-metallic impurities contained in the metal, and finally pouring said metal.

3. A method of re-melting and refining magnesium and light metal alloys containing magnesium and more particularly high percentage magnesium-base alloys, which comprises melting the metal in the presence of a thinly fluid flux containing a substantial proportion of magnesium chloride and having a melting point not substantially exceeding the melting temperature of the metal, then increasing the temperature of the metal, then stirring the metal at such elevated temperature with the said flux while adding at least one thickening agent selected from the group of metal oxides and metal fluorides in a quantity sufficient to cause inspissation of the flux already present, so as to cause said flux to combine with said inspissating agent and with the non-metallic impurities contained in the metal, and finally pouring said metal.

4. A method of re-melting and refining magnesium and light metal alloys containing magnesium and more particularly high percentage magnesium-base alloys, which comprises melting the metal in the presence of a thinly fluid flux containing a substantial proportion of magnesium chloride and having a melting point not substantially exceeding the melting temperature of the metal, then increasing the temperature of the metal, then stirring the metal at such elevated temperature with the said flux while progressively adding portions of a thickening agent in an aggregate quantity sufficient to cause inspissation of the flux already present, so as to cause said flux to combine with said inspissating agent and with the non-metallic impurities contained in the metal, and finally pouring said metal.

5. A method of re-melting and refining magnesium and light metal alloys containing magnesium and more particularly high percentage

5 magnesium-base alloys, which comprises melting the metal in the presence of a thinly fluid flux containing a substantial proportion of magnesium chloride and having a melting point not substantially exceeding the melting temperature of the metal, then increasing the temperature of the metal to at least about 720° C., then stirring the metal at such elevated temperature with the said flux while adding at least one thickening agent selected from the group of metal oxides and metal fluorides in a quantity sufficient to cause inspissation of the flux already present, so as to cause said flux to combine with said inspissating agent and with the non-metallic impurities 10 contained in the metal, and finally pouring said metal.

10 6. A method of re-melting and refining magnesium and light metal alloys containing magnesium and more particularly high percentage 15 magnesium-base alloys, which comprises melting the metal in the presence of a thinly fluid flux containing a substantial proportion of magnesium chloride and having a melting point not substantially exceeding the melting temperature 20 of the metal, then increasing the temperature of the metal, then stirring the metal at such elevated temperature with the said flux while

adding an inspissating agent comprising magnesium oxide in a quantity sufficient to cause inspissation of the flux already present, so as to cause said flux to combine with said inspissating agent and with the non-metallic impurities 5 contained in the metal, and finally pouring said metal.

7. A method of re-melting and refining magnesium and light metal alloys containing magnesium and more particularly high percentage 10 magnesium-base alloys, which comprises melting the metal in the presence of a thinly fluid saline flux having a melting point not substantially exceeding the melting temperature of the metal, then increasing the temperature of the 15 metal, then stirring the metal at such elevated temperature with the said flux while adding a thickening agent in a quantity sufficient to cause inspissation of the flux already present, so as to cause said flux to combine with said inspissating 20 agent and with the non-metallic impurities contained in the metal, establishing a protective layer of inspissated saline flux on the surface of the molten metal, heating the metal to a temperature above about 800° C., and finally allowing 25 the metal to cool to pouring temperature.

ADOLF BECK.